

## UNITED STATES PATENT OFFICE

2,288,288

## LUBRICATING OIL

Bert H. Lincoln, Ponca City, Okla., assignor, by  
mesne assignments, to Socony-Vacuum Oil  
Company, Incorporated, New York, N. Y., a cor-  
poration of New York

No Drawing. Application August 26, 1938,  
Serial No. 226,963

1 Claim. (Cl. 252--44)

This invention relates to lubricating oils and more particularly to improved lubricating oils of high film strength, high resistance to oxidation, and markedly reduced formation of corrosive products during use.

This is a continuation in part of my co-pending application, Serial No. 70163, filed March 21, 1936.

Present-day mechanical devices require lubricating oils of high film strength, of high oiliness characteristics, and of low tendency to oxidize during use. It has been found that the present-day hydrocarbon lubricants of the very highest quality are deficient in these very important characteristics. These three properties are of vital importance under conditions of thin film lubrication where the lubricant has been squeezed from between the friction surfaces because of high pressure, slow speeds, and other causes. In modern engines, large surfaces of oil are exposed to the action of atmospheric oxygen, promoting rapid oxidation. It is readily seen that the viscosity or the body of the lubricant plays no part in thin film lubrication and that the remaining film of oil must have a very high film strength and be of high oiliness value to prevent rupture of the film of the lubricant, which would cause seizure. The oil film must tend to keep the coefficient of friction as low as possible. The oil must resist oxidation when these thin films are heated in the presence of atmospheric oxygen as they are in use.

Mechanical devices are being designed for higher pressure operation, and the film strength of the best quality straight hydrocarbon lubricant has been found to be too low for satisfactory service. It will be obvious that an invention which provides a means of improving the film strength of these lubricants is of great importance to the art of lubricant manufacture and to the designer and fabricator of mechanical devices.

Substantially all machines operate in part or at times totally under conditions of boundary or thin film lubrication, under which conditions the oiliness or unctuousness of the lubricant is the first and primary requisite of efficient operation. Those skilled in the art of lubricant manufacture or machine manufacture will readily appreciate the value of an invention that will improve the oiliness of these otherwise high-quality lubricants. Furthermore, sludge and acid are especially deleterious under conditions of thin film lubrication. The sludge is not a lubricant in any sense of the word, and the soluble acid is par-

ticularly corrosive to bearing metals such as cadmium-silver, copper-lead, and the like.

In starting idle mechanical equipment which is lubricated from a sump by pumping or circulating the lubricant, there is always a short period of time in which the rubbing surfaces must operate under conditions of dry friction if ordinary hydrocarbon lubricants are used. With dry friction, the wear on friction surfaces is extreme; and during cold weather when the lubricant is sluggish or during periods when the lubricating system is not functioning properly for one reason or another, rubbing surfaces may not only suffer considerable wear but may be damaged to the point where they must be replaced. The product of this invention has a very important property of reacting with the metal surfaces, penetrating or adsorbing on the metal surfaces, and leaving a film of lubricant with high oiliness character, which remains on the metal surface irrespective of the length of time the machine has been idle.

This high oiliness film gives very even and smooth operation, which may be easily discerned by the experienced operator or lubricating engineer.

When the hydrocarbon lubricants are diluted with unburned fuel or with other light hydrocarbons, the small degree of oiliness of the original hydrocarbon lubricant is greatly decreased. It has been found that the addition of the products of this invention to hydrocarbon lubricants more than compensates for the loss in oiliness and load-carrying ability from dilution.

It is well known that, in order to obtain lubricants which are preeminently satisfactory from the standpoint of oxidation in use, it is necessary to refine the oil thoroughly and then to add an inhibitor of oxidation. The thorough refining may consist of more and heavier acid treatments or solvent treating so as to remove a considerable part of the oil and leave only the most stable portion. Such drastic refining is necessary in order to obtain stability with respect to sludge formation, but the oil is then subject to easy oxidation to form soluble acids and other corrosive materials. This can be prevented by the addition to the refined oil of small amounts of materials which either prevent the formation of these corrosive products or by some action render them inert. Furthermore, such well-refined oils are susceptible to the formation during use of lacquer-like materials which tend to stick rings. This results in blow-by and hence loss of power, failure of lubrication, scratching, scoring, overheating, and eventually replacement of parts.

It is practically impossible to refine a lubricant in such a manner as to avoid all three of these difficulties, namely, sludge, soluble corrosive products, and lacquer. It is considerably more advantageous to add the materials of this invention and avoid these difficulties by this method.

Certain compounds are adsorbed or absorbed by metals forming tenacious films at the surface of metals which are able to stand high pressures. X-ray diffraction methods have shown that compounds containing highly polar molecules, that is, molecules of unsymmetrical electrical character containing an atom or group of atoms exhibiting a secondary or residual valence, tend to produce regimentation of the molecules of hydrocarbon oil when added thereto. A metal immersed in a strongly polar compound will show a film of the compound in which there is a regimentation of molecules oriented with respect to the surface of the metal by which they are adsorbed or absorbed.

Many of these additive materials are effective when added to poorly refined or even wholly unrefined lubricants. The addends may thus be substituted in whole or in part for the usual refining processes.

In the prior art of applying these principles to the manufacture of lubricants, many diverse types of materials have been suggested to be added to obtain improvement in various characteristics. It has been found that the addition of various compounds frequently improves film strength, oxidation resistance, noncorrosiveness, and other characteristics.

One object of this invention is to provide improved inhibitors of oxidation and corrosion for addition to lubricants.

Another object of this invention is to provide film strength improving addition agents suitable for use in lubricants and especially in crankcase lubricants.

Other and further objects of this invention will appear in the course of the following description.

In general, this invention contemplates an oil of lubricating viscosity having added thereto a small amount of an organo-metallic salt. The organo-metallic salt may be an organo-metallic salt of an organic, inorganic or organo-metallic acid. Organic or inorganic salts of organo-metallic acids or organo-metallic substituted acids may be used. The organic parts of these molecules may be radicals of the aliphatic, carbocyclic, or heterocyclic series. The metallic element may be any one of a number of which the following are representative. For convenience these are listed in accordance with their occurrence in the Periodic Table.

#### Group II:

Beryllium  
Magnesium  
Zinc  
Cadmium  
Mercury

#### Group III:

Aluminum  
Thallium

#### Group IV:

Germanium  
Tin  
Lead

#### Group V:

Arsenic  
Bismuth  
Antimony

#### Group VI:

Tellurium  
Selenium

19 The compound may contain in the organic radical or attached to the metal an additional element or combination of elements including the halogens, phosphorus, sulfur, nitrogen or oxygen.

15 The organo-metallic salts of this invention have a dual action in a lubricant. One action involves increased load-carrying ability and/or oiliness, while another action is directed to the stability of the lubricant. For load-carrying capacity, quantities ranging from 0.1 per cent to about 10 per cent may be added. As an anti-corrosive agent and/or an anti-sludging agent, much smaller amounts may be required ranging from approximately 0.001 to 0.1 per cent. The action of the organo-metallic salts is specific but difficult to understand. These compounds may be added to any type of hydrocarbon lubricants but show an unusual value in highly refined and solvent treated lubricants. By oil having lubricating viscosity in the appended claim, it is meant to include the so-called mineral oils and various hydrogenated, polymerized and otherwise synthetically treated oils such as voltolized oils, aluminum chloride treated oils, and the like. Furthermore the lubricating oil may consist in whole or in part of shale oil, animal or vegetable oils such as castor oil, lard oil, corn oil, cottonseed oil, and the like.

30 In practice, it is better to employ compounds whose boiling point is above 225° F. in order that the addition compound will not be evaporated or distilled in use. The selection of a particular compound or compounds to be used as an addition agent to the hydrocarbon or other oil is to be made considering the physical and chemical properties of the various compounds and the use to which the blend is put. Thus, if water is likely to be present during use, a salt or combination of salts is selected which is not affected by water. If a particular added compound proves too volatile for its application, a higher boiling material should be used and the more volatile compound used for blending in an oil intended for duty at lower temperatures. In general, for automotive crankcase lubricants, it is preferred to use compounds having vapor pressures of less than atmospheric at 250° F.

35 The following compounds may be used in accordance with this invention. All and each of these are to be considered as examples of this invention when blended in an oil of lubricating viscosity.

#### I. Organo-metallic salts of inorganic acids

##### A. Salts of acids of nitrogen

40 1. Salts of nitrous acid  
Triamyltin nitrite  $(C_5H_{11})_3SnNO_2$   
Tribenzyltin nitrite  
 $(C_6H_5CH_2)_3SnNO_2$   
Tripyridyl germanium nitrite  
 $(C_5H_4N)_3GeNO_2$   
70 Trithienyltin nitrite  $(C_4H_3S)_3SnNO_2$   
Furfurylmercuric nitrite  
 $(C_4H_3O)HgNO_2$   
Di-isoamylaluminum nitrite  
 $(C_5H_{11})_2AlNO_2$

|                                                                                                                                                                        |    |                                                                                                                                                                                                                                                                                |
|------------------------------------------------------------------------------------------------------------------------------------------------------------------------|----|--------------------------------------------------------------------------------------------------------------------------------------------------------------------------------------------------------------------------------------------------------------------------------|
| Di-phenylbismuth nitrite<br>(C <sub>6</sub> H <sub>5</sub> ) <sub>2</sub> BiNO <sub>2</sub>                                                                            |    | Chloronaphthylmercuric phosphate<br>(ClC <sub>10</sub> H <sub>6</sub> Hg) <sub>3</sub> PO <sub>4</sub>                                                                                                                                                                         |
| o-Tolyltellurium nitrite<br>(CH <sub>3</sub> C <sub>6</sub> H <sub>4</sub> )TeNO <sub>2</sub>                                                                          |    | Dibenzothienylantimony phosphate<br>(C <sub>12</sub> H <sub>7</sub> S.Sb) <sub>3</sub> (PO <sub>4</sub> ) <sub>2</sub>                                                                                                                                                         |
| Tri-omega-chloroamyltin nitrite 5<br>(ClC <sub>5</sub> H <sub>10</sub> ) <sub>3</sub> SnNO <sub>2</sub>                                                                |    | Allyl diamyltin diallyltin phosphate<br>[(C <sub>3</sub> H <sub>5</sub> ) <sub>2</sub> C <sub>5</sub> H <sub>11</sub> ) <sub>2</sub> Sn]<br>[(C <sub>3</sub> H <sub>5</sub> ) <sub>2</sub> Sn] <sub>2</sub> PO <sub>4</sub>                                                    |
| n-Butylberyllium nitrite C <sub>4</sub> H <sub>9</sub> BeNO <sub>2</sub>                                                                                               |    | Tribenzyltin diresylphosphate<br>[(C <sub>6</sub> H <sub>5</sub> CH <sub>2</sub> ) <sub>3</sub> Sn] <sub>2</sub> (CH <sub>3</sub> C <sub>6</sub> H <sub>4</sub> ) <sub>2</sub> PO <sub>4</sub>                                                                                 |
| 2. Salts of nitric acid                                                                                                                                                |    | Di-p-nitrophenylin phosphate<br>[(O <sub>2</sub> NC <sub>6</sub> H <sub>4</sub> ) <sub>2</sub> Sn] <sub>3</sub> (PO <sub>4</sub> ) <sub>2</sub>                                                                                                                                |
| Diethylthallium nitrate<br>(C <sub>2</sub> H <sub>5</sub> ) <sub>2</sub> TlNO <sub>3</sub>                                                                             | 10 | Tri (4-benzoylphenyl) lead phosphate<br>[(C <sub>6</sub> H <sub>5</sub> CO C <sub>6</sub> H <sub>4</sub> ) <sub>3</sub> Pb] <sub>3</sub> PO <sub>4</sub>                                                                                                                       |
| Trilauryl tin nitrate (C <sub>12</sub> H <sub>25</sub> ) <sub>3</sub> SnNO <sub>3</sub>                                                                                |    | 2-Ethylhexylzinc phosphate<br>[C <sub>4</sub> H <sub>9</sub> CH(C <sub>2</sub> H <sub>5</sub> )CH <sub>2</sub> Zn] <sub>3</sub> PO <sub>4</sub>                                                                                                                                |
| Di-p-tolyl lead dinitrate<br>(CH <sub>3</sub> C <sub>6</sub> H <sub>4</sub> ) <sub>2</sub> Pb(NO <sub>3</sub> ) <sub>2</sub>                                           |    | n-Butylberyllium phosphate<br>(C <sub>4</sub> H <sub>9</sub> Be) <sub>3</sub> PO <sub>4</sub>                                                                                                                                                                                  |
| Benzyl cadmium nitrate<br>C <sub>6</sub> H <sub>5</sub> CH <sub>2</sub> CdNO <sub>3</sub>                                                                              | 15 | Diphenyllead phosphate<br>[(C <sub>6</sub> H <sub>5</sub> ) <sub>2</sub> Pb] <sub>3</sub> (PO <sub>4</sub> ) <sub>2</sub>                                                                                                                                                      |
| p-tert-Butylphenylarsenic nitrate<br>C <sub>4</sub> H <sub>9</sub> C <sub>6</sub> H <sub>4</sub> AsNO <sub>3</sub>                                                     |    | Tribenzyltin monohydrogen phosphate<br>[(C <sub>6</sub> H <sub>5</sub> CH <sub>2</sub> ) <sub>3</sub> Sn] <sub>2</sub> HPO <sub>4</sub>                                                                                                                                        |
| p-Aminobenzylselenium nitrate<br>H <sub>2</sub> NC <sub>6</sub> H <sub>4</sub> CH <sub>2</sub> SeNO <sub>3</sub>                                                       |    | Tribenzyltin dihydrogen phosphate<br>[(C <sub>6</sub> H <sub>5</sub> CH <sub>2</sub> ) <sub>3</sub> Sn] <sub>2</sub> H <sub>2</sub> PO <sub>4</sub>                                                                                                                            |
| Pyridyl cyclohexyl germanium dinitrate (C <sub>5</sub> H <sub>4</sub> N)(C <sub>6</sub> H <sub>11</sub> )Ge(NO <sub>3</sub> ) <sub>2</sub>                             | 20 | Diethylthallium phosphate<br>[(C <sub>2</sub> H <sub>5</sub> ) <sub>2</sub> Tl] <sub>3</sub> PO <sub>4</sub>                                                                                                                                                                   |
| Diamyl tin dinitrate<br>(C <sub>5</sub> H <sub>11</sub> ) <sub>2</sub> Sn(NO <sub>3</sub> ) <sub>2</sub>                                                               |    | 4. Salts of thiophosphoric acids                                                                                                                                                                                                                                               |
| Tri-omega-chloroamyltin nitrate<br>(ClC <sub>5</sub> H <sub>10</sub> ) <sub>3</sub> SnNO <sub>3</sub>                                                                  | 25 | Triamyltin monothiophosphate<br>[(C <sub>5</sub> H <sub>11</sub> ) <sub>3</sub> Sn] <sub>3</sub> PO <sub>3</sub> S                                                                                                                                                             |
| n-Butylberyllium nitrate C <sub>4</sub> H <sub>9</sub> BeNO <sub>3</sub>                                                                                               |    | Tribenzyltin monothiophosphate<br>[(C <sub>6</sub> H <sub>5</sub> CH <sub>2</sub> ) <sub>3</sub> Sn] <sub>3</sub> PO <sub>3</sub> S                                                                                                                                            |
| B. Salts of acids of phosphorus                                                                                                                                        |    | Tribenzyltin dithiophosphate<br>[(C <sub>6</sub> H <sub>5</sub> CH <sub>2</sub> ) <sub>3</sub> Sn] <sub>3</sub> PO <sub>2</sub> S <sub>2</sub>                                                                                                                                 |
| 1. Salts of phosphorous acid                                                                                                                                           |    | Tribenzyltin trithiophosphate<br>[(C <sub>6</sub> H <sub>5</sub> CH <sub>2</sub> ) <sub>3</sub> Sn] <sub>3</sub> POS <sub>3</sub>                                                                                                                                              |
| Tribenzyltin phosphite<br>[(C <sub>6</sub> H <sub>5</sub> CH <sub>2</sub> ) <sub>3</sub> Sn] <sub>3</sub> PO <sub>3</sub>                                              | 30 | Tribenzyltin tetrathiophosphate<br>[(C <sub>6</sub> H <sub>5</sub> CH <sub>2</sub> ) <sub>3</sub> Sn] <sub>3</sub> PS <sub>4</sub>                                                                                                                                             |
| Triamyltin phosphite<br>[(C <sub>5</sub> H <sub>11</sub> ) <sub>3</sub> Sn] <sub>3</sub> PO <sub>3</sub>                                                               |    | Di-beta-ethoxyethylthallium monothiophosphate<br>[(C <sub>2</sub> H <sub>5</sub> O C <sub>2</sub> H <sub>4</sub> ) <sub>2</sub> Tl] <sub>3</sub> PO <sub>3</sub> S                                                                                                             |
| Tripyridyltin phosphite<br>[(C <sub>5</sub> H <sub>4</sub> N) <sub>3</sub> Sn] <sub>3</sub> PO <sub>3</sub>                                                            |    | beta - Hydroxyethylmercury tetrathiophosphate (HOCH <sub>2</sub> Hg) <sub>3</sub> PS <sub>4</sub>                                                                                                                                                                              |
| Di-omega-chloroamyltin phosphite 35<br>[(ClC <sub>5</sub> H <sub>10</sub> ) <sub>2</sub> Sn] <sub>3</sub> (PO <sub>3</sub> ) <sub>2</sub>                              |    | omega-Chloroamylantimony dithiophosphate (ClC <sub>5</sub> H <sub>10</sub> Sb) <sub>3</sub> (PO <sub>2</sub> S <sub>2</sub> ) <sub>2</sub>                                                                                                                                     |
| o-Tolylzinc phosphite<br>(CH <sub>3</sub> C <sub>6</sub> H <sub>4</sub> Zn) <sub>3</sub> PO <sub>3</sub>                                                               |    | p - Aminophenylselenium trithiophosphate (H <sub>2</sub> NC <sub>6</sub> H <sub>4</sub> Se) <sub>3</sub> POS <sub>3</sub>                                                                                                                                                      |
| beta-Thioethylthallium phosphite<br>(HSC <sub>2</sub> H <sub>4</sub> Tl) <sub>3</sub> (PO <sub>3</sub> ) <sub>2</sub>                                                  | 40 | beta-Mercapto-alpha - naphthylbismuth monothiophosphate<br>(HS.C <sub>10</sub> H <sub>8</sub> Bi) <sub>3</sub> (PO <sub>3</sub> S) <sub>2</sub>                                                                                                                                |
| Tribenzyltin diresylphosphate<br>[(C <sub>6</sub> H <sub>5</sub> CH <sub>2</sub> ) <sub>3</sub> Sn] <sub>2</sub> PO <sub>4</sub>                                       |    | Pyridyl cyclohexyltin dipyridyl cyclohexyltin monothiophosphate<br>[(C <sub>5</sub> H <sub>4</sub> N) <sub>2</sub> (C <sub>6</sub> H <sub>11</sub> )Sn]<br>[(C <sub>5</sub> H <sub>4</sub> N) <sub>2</sub> (C <sub>6</sub> H <sub>11</sub> )Sn] <sub>2</sub> PO <sub>3</sub> S |
| Diaryl tin dithiophosphate<br>[(C <sub>5</sub> H <sub>11</sub> ) <sub>2</sub> Sn] <sub>3</sub> (PO <sub>2</sub> S) <sub>2</sub>                                        | 50 | Tribenzyltin monohydrogen dithiophosphate<br>[(C <sub>6</sub> H <sub>5</sub> CH <sub>2</sub> ) <sub>3</sub> Sn] <sub>2</sub> HPO <sub>2</sub> S <sub>2</sub>                                                                                                                   |
| Trilauryltin trithiophosphate<br>[(C <sub>12</sub> H <sub>25</sub> ) <sub>3</sub> Sn] <sub>3</sub> PS <sub>3</sub>                                                     |    | n - Butylberyllium tetrathiophosphate (C <sub>4</sub> H <sub>9</sub> Be) <sub>3</sub> PS <sub>4</sub>                                                                                                                                                                          |
| Allyl dicyclohexyltin monothiophosphate<br>(C <sub>3</sub> H <sub>5</sub> )(C <sub>6</sub> H <sub>11</sub> ) <sub>2</sub> Sn] <sub>3</sub> PO <sub>2</sub> S           | 55 | 5. Salts of pyrophosphoric acid                                                                                                                                                                                                                                                |
| p - Amyloxyphenylthallium trithiophosphate (C <sub>5</sub> H <sub>11</sub> O.C <sub>6</sub> H <sub>4</sub> Tl) <sub>3</sub> (PS <sub>3</sub> ) <sub>2</sub>            |    | Trilauryltin pyrophosphate<br>[(C <sub>12</sub> H <sub>25</sub> ) <sub>3</sub> Sn] <sub>4</sub> P <sub>2</sub> O <sub>7</sub>                                                                                                                                                  |
| Thienylmercuric dithiophosphate<br>(C <sub>4</sub> H <sub>9</sub> S.Hg) <sub>3</sub> POS <sub>2</sub>                                                                  |    | Tribenzyltin pyrophosphate<br>[(C <sub>6</sub> H <sub>5</sub> CH <sub>2</sub> ) <sub>3</sub> Sn] <sub>4</sub> P <sub>2</sub> O <sub>7</sub>                                                                                                                                    |
| omega-Chloroamylselenium mono- 60<br>thiophosphate (ClC <sub>5</sub> H <sub>10</sub> Se) <sub>3</sub> PO <sub>2</sub> S                                                |    | Tribenzyltin dicyclohexyltin monohydrogen pyrophosphate<br>[(C <sub>6</sub> H <sub>5</sub> CH <sub>2</sub> ) <sub>3</sub> Sn]<br>[(C <sub>6</sub> H <sub>11</sub> ) <sub>2</sub> Sn] <sub>2</sub> HP <sub>2</sub> O <sub>7</sub>                                               |
| p-Dimethylaminophenylbismuth tri-<br>thiophosphate<br>[(CH <sub>3</sub> ) <sub>2</sub> NC <sub>6</sub> H <sub>4</sub> Bi] <sub>3</sub> (PS <sub>3</sub> ) <sub>2</sub> |    | Furfurylmercuric pyrophosphate<br>(C <sub>4</sub> H <sub>9</sub> O.Hg) <sub>4</sub> P <sub>2</sub> O <sub>7</sub>                                                                                                                                                              |
| Tribenzyltin monohydrogen mono- 65<br>thiophosphate<br>[(C <sub>6</sub> H <sub>5</sub> CH <sub>2</sub> ) <sub>3</sub> Sn] <sub>2</sub> HPO <sub>2</sub> S              |    | Di (4-trichloronaphthoylnaphthyl)<br>thallium pyrophosphate<br>[(Cl <sub>3</sub> C <sub>10</sub> H <sub>4</sub> COCl <sub>10</sub> H <sub>6</sub> ) <sub>2</sub> Tl] <sub>4</sub> P <sub>2</sub> O <sub>7</sub>                                                                |
| n - Butylberyllium monothiophos-<br>phite (C <sub>4</sub> H <sub>9</sub> Be) <sub>3</sub> PO <sub>2</sub> S                                                            | 70 | Allylthallium dihydrogen pyrophosphate<br>C <sub>3</sub> H <sub>5</sub> TlH <sub>2</sub> P <sub>2</sub> O <sub>7</sub>                                                                                                                                                         |
| 3. Salts of phosphoric acid                                                                                                                                            |    |                                                                                                                                                                                                                                                                                |
| Tribenzyltin phosphate<br>[(C <sub>6</sub> H <sub>5</sub> CH <sub>2</sub> ) <sub>3</sub> Sn] <sub>3</sub> PO <sub>4</sub>                                              |    |                                                                                                                                                                                                                                                                                |
| Pyridyl cyclohexylthallium phos-<br>phate [(C <sub>5</sub> H <sub>4</sub> N)(C <sub>6</sub> H <sub>11</sub> )Tl] <sub>3</sub> PO <sub>4</sub>                          | 75 |                                                                                                                                                                                                                                                                                |

|                                                                                                                                                                                            |    |                                                                                                                                                                                                               |
|--------------------------------------------------------------------------------------------------------------------------------------------------------------------------------------------|----|---------------------------------------------------------------------------------------------------------------------------------------------------------------------------------------------------------------|
| Dicetylarsenic pyrophosphate<br>[(C <sub>16</sub> H <sub>33</sub> ) <sub>2</sub> As] <sub>4</sub> P <sub>2</sub> O <sub>7</sub>                                                            |    | Tribenzyltin hydrogen hypophosphate (C <sub>6</sub> H <sub>5</sub> CH <sub>2</sub> ) <sub>3</sub> SnHPO <sub>3</sub>                                                                                          |
| Tritiylselenium dihydrogen pyro-<br>phosphate [(C <sub>6</sub> H <sub>5</sub> ) <sub>3</sub> C.Se] <sub>2</sub> H <sub>2</sub> P <sub>2</sub> O <sub>7</sub>                               |    | Trilauryltin hypophosphate [(C <sub>12</sub> H <sub>25</sub> ) <sub>3</sub> Sn] <sub>2</sub> PO <sub>3</sub>                                                                                                  |
| p-Nitrobenzeneazophenylzinc pyro-<br>phosphate<br>(O <sub>2</sub> N.C <sub>6</sub> H <sub>4</sub> N=N.C <sub>6</sub> H <sub>4</sub> Zn) <sub>4</sub> P <sub>2</sub> O <sub>7</sub>         | 5  | Dithienylead hypophosphate (C <sub>4</sub> H <sub>3</sub> S) <sub>2</sub> PbPO <sub>3</sub>                                                                                                                   |
| n-Butylberyllium pyrophosphate<br>(C <sub>4</sub> H <sub>9</sub> Be) <sub>4</sub> P <sub>2</sub> O <sub>7</sub>                                                                            |    | Divinylthallium hypophosphate [(CH <sub>2</sub> =CH-) <sub>2</sub> Tl] <sub>2</sub> PO <sub>3</sub>                                                                                                           |
| 6. Salts of metaphosphoric acid and its<br>polymers                                                                                                                                        | 10 | Oleylphenylmercuric hypophos-<br>phate (C <sub>18</sub> H <sub>35</sub> C <sub>6</sub> H <sub>4</sub> Hg.) <sub>2</sub> PO <sub>3</sub>                                                                       |
| Triamyltin monometaphosphate<br>(C <sub>6</sub> H <sub>11</sub> ) <sub>3</sub> SnPO <sub>3</sub>                                                                                           |    | Lauroylphenylarsenic hypophos-<br>phate C <sub>11</sub> H <sub>22</sub> CO <sub>6</sub> H <sub>4</sub> AsPO <sub>3</sub>                                                                                      |
| Tribenzyltin monometaphosphate<br>(C <sub>6</sub> H <sub>5</sub> CH <sub>2</sub> ) <sub>3</sub> SnPO <sub>3</sub>                                                                          | 15 | 2-ethylhexyltellurium hydrogen hy-<br>poprophosphate<br>C <sub>4</sub> H <sub>9</sub> CH(C <sub>2</sub> H <sub>5</sub> )CH <sub>2</sub> TeHPO <sub>3</sub>                                                    |
| Dicinnamyltin monometaphosphate<br>[(C <sub>6</sub> H <sub>5</sub> CH=CHCH <sub>2</sub> ( <sub>2</sub> Sn)(PO <sub>3</sub> ) <sub>2</sub>                                                  |    | omega-Chloroamylbismuth hypo-<br>phosphate ClC <sub>5</sub> H <sub>10</sub> BiPO <sub>3</sub>                                                                                                                 |
| Tri (4-methylcyclohexyl) tin mono-<br>metaphosphate<br>(CH <sub>3</sub> C <sub>6</sub> H <sub>10</sub> ) <sub>3</sub> SnPO <sub>3</sub>                                                    | 20 | Di (thiobenzoylphenyl) indium hy-<br>poprophosphate<br>[(C <sub>6</sub> H <sub>5</sub> CS.C <sub>6</sub> H <sub>4</sub> ) <sub>2</sub> In] <sub>2</sub> PO <sub>3</sub>                                       |
| Dibenzofurylmercuric monometa-<br>phosphate C <sub>12</sub> H <sub>7</sub> OHgPO <sub>3</sub>                                                                                              |    | n-Butylberyllium hypophosphate<br>(C <sub>4</sub> H <sub>9</sub> Be) <sub>2</sub> PO <sub>3</sub>                                                                                                             |
| Di (p-mercaptophenyl) aluminum<br>monometaphosphate<br>(HSC <sub>6</sub> H <sub>4</sub> C <sub>6</sub> H <sub>4</sub> ) <sub>2</sub> AlPO <sub>3</sub>                                     | 25 | C. Salts of acids of sulfur                                                                                                                                                                                   |
| Pentacosylphenylantimony mono-<br>metaphosphate<br>C <sub>25</sub> H <sub>51</sub> C <sub>6</sub> H <sub>4</sub> Sb(PO <sub>3</sub> ) <sub>2</sub>                                         |    | 1. Salts of hydrogen sulfide                                                                                                                                                                                  |
| Trityltellurium monometaphosphate<br>(C <sub>6</sub> H <sub>5</sub> ) <sub>3</sub> C.TePO <sub>3</sub>                                                                                     | 30 | Tribenzyltin sulfide<br>[(C <sub>6</sub> H <sub>5</sub> CH <sub>2</sub> ) <sub>3</sub> Sn] <sub>2</sub> S                                                                                                     |
| Tribenzyltin dimetaphosphate<br>[(C <sub>6</sub> H <sub>5</sub> CH <sub>2</sub> ) <sub>3</sub> Sn] <sub>2</sub> P <sub>2</sub> O <sub>6</sub>                                              |    | Tribenzyltin hydrosulfide<br>(C <sub>6</sub> H <sub>5</sub> CH <sub>2</sub> ) <sub>3</sub> SnSH                                                                                                               |
| Tribenzyltin trimetaphosphate<br>[(C <sub>6</sub> H <sub>5</sub> CH <sub>2</sub> ) <sub>3</sub> Sn] <sub>3</sub> P <sub>3</sub> O <sub>9</sub>                                             |    | Tribenzyltin benzyl sulfide<br>(C <sub>6</sub> H <sub>5</sub> CH <sub>2</sub> ) <sub>3</sub> SnSCH <sub>2</sub> C <sub>6</sub> H <sub>5</sub>                                                                 |
| Tribenzyltin tetrametaphosphate<br>[(C <sub>6</sub> H <sub>5</sub> CH <sub>2</sub> ) <sub>3</sub> Sn] <sub>4</sub> P <sub>4</sub> O <sub>12</sub>                                          | 35 | Trilauryltin sulfide [(C <sub>12</sub> H <sub>25</sub> ) <sub>3</sub> Sn] <sub>2</sub> S                                                                                                                      |
| Tribenzyltin pentametaphosphate<br>[(C <sub>6</sub> H <sub>5</sub> CH <sub>2</sub> ) <sub>3</sub> Sn] <sub>5</sub> P <sub>5</sub> O <sub>15</sub>                                          |    | Dilauryltin sulfide [(C <sub>12</sub> H <sub>25</sub> ) <sub>3</sub> Sn]S                                                                                                                                     |
| Tribenzyltin hexametaphosphate<br>[(C <sub>6</sub> H <sub>5</sub> CH <sub>2</sub> ) <sub>3</sub> Sn] <sub>6</sub> P <sub>6</sub> O <sub>18</sub>                                           | 40 | Lauryltin sulfide (C <sub>12</sub> H <sub>25</sub> Sn) <sub>2</sub> S <sub>3</sub>                                                                                                                            |
| n-Butylberyllium dimetaphosphate<br>(C <sub>4</sub> H <sub>9</sub> Be) <sub>2</sub> P <sub>2</sub> O <sub>6</sub>                                                                          |    | Lauryltin hydrosulfide<br>C <sub>12</sub> H <sub>25</sub> Sn(SH) <sub>3</sub>                                                                                                                                 |
| 7. Salts of hypophosphorous acid                                                                                                                                                           |    | Di(ethylcyclohexyl) thallium sulfide<br>[(C <sub>2</sub> H <sub>5</sub> C <sub>6</sub> H <sub>10</sub> ) <sub>2</sub> Tl] <sub>2</sub> S                                                                      |
| Tribenzyltin hypophosphite<br>[(C <sub>6</sub> H <sub>5</sub> CH <sub>2</sub> ) <sub>3</sub> Sn] <sub>3</sub> PO <sub>2</sub>                                                              | 45 | Octadecyllead sulfide (C <sub>18</sub> H <sub>37</sub> Pb) <sub>2</sub> S                                                                                                                                     |
| Tribenzyltin monohydrogen hypo-<br>phosphite [(C <sub>6</sub> H <sub>5</sub> CH <sub>2</sub> ) <sub>3</sub> Sn] <sub>2</sub> HPO <sub>2</sub>                                              |    | Tri-octadecyllead sulfide<br>[(C <sub>18</sub> H <sub>37</sub> ) <sub>3</sub> Pb] <sub>2</sub> S                                                                                                              |
| Tribenzyltin dihydrogen hypophos-<br>phite (C <sub>6</sub> H <sub>5</sub> CH <sub>2</sub> ) <sub>3</sub> SnH <sub>2</sub> PO <sub>2</sub>                                                  |    | Tripentacosyllead sulfide<br>[(C <sub>25</sub> H <sub>51</sub> ) <sub>3</sub> Pb] <sub>2</sub> S                                                                                                              |
| Crotonylmagnesium hypophosphite<br>(CH <sub>3</sub> CH=CHCH <sub>2</sub> Mg) <sub>3</sub> PO <sub>2</sub>                                                                                  | 50 | Triquinolyltin triauryltin sulfide<br>[(C <sub>6</sub> H <sub>5</sub> N) <sub>3</sub> Sn] <sub>2</sub> [(C <sub>12</sub> H <sub>25</sub> ) <sub>3</sub> Sn]S                                                  |
| Cycloamyl amyliundium hypophos-<br>phite [(C <sub>5</sub> H <sub>9</sub> )(C <sub>5</sub> H <sub>11</sub> )In] <sub>3</sub> PO <sub>2</sub>                                                |    | Methacrylylselenium sulfide<br>(CH <sub>2</sub> =C(CH <sub>3</sub> )CH <sub>2</sub> Se) <sub>2</sub> S                                                                                                        |
| Cycloamylindium hypophosphite<br>(C <sub>5</sub> H <sub>9</sub> In) <sub>3</sub> PO <sub>2</sub>                                                                                           | 55 | Diamylantimony sulfide<br>[(C <sub>5</sub> H <sub>11</sub> ) <sub>2</sub> Sb] <sub>2</sub> S                                                                                                                  |
| omega-Chloroamyl ethyltin hypo-<br>phosphite<br>[(ClC <sub>5</sub> H <sub>10</sub> )(C <sub>2</sub> H <sub>5</sub> )Sn] <sub>3</sub> (PO <sub>2</sub> ) <sub>2</sub>                       |    | Diphenyllead sulfide (C <sub>6</sub> H <sub>5</sub> ) <sub>2</sub> PbS                                                                                                                                        |
| Tri (triethylstannyl) tin hypophos-<br>phite [(C <sub>2</sub> H <sub>5</sub> ) <sub>3</sub> Sn] <sub>3</sub> Sn] <sub>3</sub> PO <sub>2</sub>                                              | 60 | n-Butylberyllium sulfide<br>(C <sub>4</sub> H <sub>9</sub> Be) <sub>2</sub> S                                                                                                                                 |
| Tripyridyltin hypophosphite<br>[(C <sub>5</sub> H <sub>4</sub> N) <sub>3</sub> Sn] <sub>3</sub> PO <sub>2</sub>                                                                            |    | 2. Salts of sulfurous acid                                                                                                                                                                                    |
| Trilauryltin hypophosphite<br>[(C <sub>12</sub> H <sub>25</sub> ) <sub>3</sub> Sn] <sub>3</sub> PO <sub>2</sub>                                                                            |    | Tribenzyltin sulfite<br>[(C <sub>6</sub> H <sub>5</sub> CH <sub>2</sub> ) <sub>3</sub> Sn] <sub>2</sub> SO <sub>3</sub>                                                                                       |
| omega-Diethylbismuthylamylbis-<br>methyl hypophosphite<br>(C <sub>2</sub> H <sub>5</sub> ) <sub>2</sub> Bi(CH <sub>2</sub> ) <sub>5</sub> Bi] <sub>3</sub> (PO <sub>2</sub> ) <sub>2</sub> | 65 | Tribenzyltin hydrosulfite<br>(C <sub>6</sub> H <sub>5</sub> CH <sub>2</sub> ) <sub>3</sub> SnSO <sub>3</sub> H                                                                                                |
| Amylseelenium hypophosphite<br>(C <sub>5</sub> H <sub>11</sub> Se) <sub>3</sub> PO <sub>2</sub>                                                                                            |    | Tribenzyltin dibenzylthallium sulfite<br>[(C <sub>6</sub> H <sub>5</sub> CH <sub>2</sub> ) <sub>3</sub> Sn]<br>[(C <sub>6</sub> H <sub>5</sub> CH <sub>2</sub> ) <sub>2</sub> Tl]SO <sub>3</sub>              |
| n-Butylberyllium hypophosphite<br>(C <sub>4</sub> H <sub>9</sub> Be) <sub>3</sub> PO <sub>2</sub>                                                                                          | 70 | Thienylzinc sulfite (C <sub>4</sub> H <sub>3</sub> SZn) <sub>2</sub> SO <sub>3</sub>                                                                                                                          |
| 8. Salts of hypophosphoric acid                                                                                                                                                            |    | omega-Chloroamylarsenic sulfite<br>ClC <sub>5</sub> H <sub>10</sub> AsSO <sub>3</sub>                                                                                                                         |
| Tribenzyltin hypophosphate<br>[(C <sub>6</sub> H <sub>5</sub> CH <sub>2</sub> ) <sub>3</sub> Sn] <sub>2</sub> PO <sub>3</sub>                                                              | 75 | n-Butylberyllium sulfite<br>(C <sub>4</sub> H <sub>9</sub> Be) <sub>2</sub> SO <sub>3</sub>                                                                                                                   |
|                                                                                                                                                                                            |    | Allsylselenium sulfite (C <sub>3</sub> H <sub>5</sub> Se) <sub>2</sub> SO <sub>3</sub>                                                                                                                        |
|                                                                                                                                                                                            |    | Tribenzyltin amyl sulfite<br>(C <sub>6</sub> H <sub>5</sub> CH <sub>2</sub> ) <sub>3</sub> SnSO <sub>3</sub> C <sub>5</sub> H <sub>11</sub>                                                                   |
|                                                                                                                                                                                            |    | 3. Salts of sulfuric acid                                                                                                                                                                                     |
|                                                                                                                                                                                            |    | Tribenzyltin sulfate<br>[(C <sub>6</sub> H <sub>5</sub> CH <sub>2</sub> ) <sub>3</sub> Sn] <sub>2</sub> SO <sub>4</sub>                                                                                       |
|                                                                                                                                                                                            |    | Dibenzyltin sulfate<br>(C <sub>6</sub> H <sub>5</sub> CH <sub>2</sub> ) <sub>2</sub> SnSO <sub>4</sub>                                                                                                        |
|                                                                                                                                                                                            |    | Tribenzyltin tri-p-tolyllead sulfate<br>[(C <sub>6</sub> H <sub>5</sub> CH <sub>2</sub> ) <sub>3</sub> Sn]<br>[(CH <sub>3</sub> C <sub>6</sub> H <sub>4</sub> ) <sub>3</sub> Pb] <sub>2</sub> SO <sub>4</sub> |

|                                                                                                                                                                                                 |    |                                                                                                                                                                                                                                                                |
|-------------------------------------------------------------------------------------------------------------------------------------------------------------------------------------------------|----|----------------------------------------------------------------------------------------------------------------------------------------------------------------------------------------------------------------------------------------------------------------|
| Benzyl cadmium sulfate<br>(C <sub>6</sub> H <sub>5</sub> CH <sub>2</sub> Cd) <sub>2</sub> SO <sub>4</sub>                                                                                       |    | Tribenzyltin carbonate<br>CO[OSn(CH <sub>2</sub> C <sub>6</sub> H <sub>5</sub> ) <sub>3</sub> ] <sub>2</sub>                                                                                                                                                   |
| Tri-omega-chloroamyllead sulfate<br>[(ClC <sub>5</sub> H <sub>10</sub> ) <sub>3</sub> Pb] <sub>2</sub> SO <sub>4</sub>                                                                          |    | Dilauryltin oleate<br>(C <sub>17</sub> H <sub>33</sub> CO <sub>2</sub> ) <sub>2</sub> Sn(C <sub>12</sub> H <sub>25</sub> ) <sub>2</sub>                                                                                                                        |
| Tribenzyltin hydrogen sulfate<br>(C <sub>6</sub> H <sub>5</sub> CH <sub>2</sub> ) <sub>3</sub> SnHSO <sub>4</sub>                                                                               | 5  | Lauryltin oleate<br>(C <sub>17</sub> H <sub>33</sub> CO <sub>2</sub> ) <sub>3</sub> SnC <sub>12</sub> H <sub>25</sub>                                                                                                                                          |
| Tribenzyltin amyl sulfate<br>[(C <sub>6</sub> H <sub>5</sub> CH <sub>2</sub> ) <sub>3</sub> Sn] <sub>2</sub> C <sub>5</sub> H <sub>11</sub> SO <sub>4</sub>                                     |    | Dicyclohexylarsenic oleate<br>C <sub>17</sub> H <sub>33</sub> CO <sub>2</sub> As(C <sub>6</sub> H <sub>11</sub> ) <sub>2</sub>                                                                                                                                 |
| p-tert.-Butylphenylindium (III) sulfate<br>C <sub>4</sub> H <sub>9</sub> C <sub>6</sub> H <sub>4</sub> InSO <sub>4</sub>                                                                        | 10 | Allylselenium oleate<br>C <sub>17</sub> H <sub>33</sub> CO <sub>2</sub> SeC <sub>3</sub> H <sub>5</sub>                                                                                                                                                        |
| p-tert.-Butylphenylindium (II) sulfate<br>(C <sub>4</sub> H <sub>9</sub> C <sub>6</sub> H <sub>4</sub> In) <sub>2</sub> SO <sub>4</sub>                                                         |    | n-Butylberyllium oleate<br>C <sub>4</sub> H <sub>9</sub> BeO.CO.C <sub>17</sub> H <sub>33</sub>                                                                                                                                                                |
| Di-p-aminobenzylbismuth sulfate<br>[(H <sub>2</sub> N <sub>2</sub> C <sub>6</sub> H <sub>4</sub> CH <sub>2</sub> ) <sub>2</sub> Bi] <sub>2</sub> SO <sub>4</sub>                                |    | Dilauryltin oleate ethyl succinate<br>(C <sub>17</sub> H <sub>33</sub> CO <sub>2</sub> ) <sub>2</sub> Sn(C <sub>12</sub> H <sub>25</sub> ) <sub>2</sub><br>CH <sub>2</sub> CH <sub>2</sub> CO <sub>2</sub> ) Sn(C <sub>12</sub> H <sub>25</sub> ) <sub>2</sub> |
| Pyridyl dicyclohexyltin sulfate<br>[(C <sub>5</sub> H <sub>4</sub> N)(C <sub>6</sub> H <sub>11</sub> ) <sub>2</sub> Sn] <sub>2</sub> SO <sub>4</sub>                                            | 15 | Pyridyl diethyllead oleate<br>C <sub>17</sub> H <sub>33</sub> CO <sub>2</sub> [Pb(C <sub>2</sub> H <sub>5</sub> ) <sub>2</sub> (C <sub>5</sub> H <sub>4</sub> N)]                                                                                              |
| Tri(mercaptop-tolyl) lead sulfate<br>[(HSC <sub>6</sub> H <sub>5</sub> CH <sub>3</sub> ) <sub>3</sub> Pb] <sub>2</sub> SO <sub>4</sub>                                                          |    | p-tert.-Butylphenylzinc oleate<br>C <sub>17</sub> H <sub>33</sub> CO <sub>2</sub> ZnC <sub>6</sub> H <sub>4</sub> C <sub>4</sub> H <sub>9</sub>                                                                                                                |
| n-Butylberyllium sulfate<br>(C <sub>4</sub> H <sub>9</sub> Be) <sub>2</sub> SO <sub>4</sub>                                                                                                     | 20 | Di-alpha-amino-beta-naphthylindium oleate<br>C <sub>17</sub> H <sub>33</sub> CO <sub>2</sub> In(C <sub>10</sub> H <sub>6</sub> NH <sub>2</sub> ) <sub>2</sub>                                                                                                  |
| 4. Thiosulfates                                                                                                                                                                                 |    | iso-Propylmercuric stearate<br>C <sub>17</sub> H <sub>35</sub> CO <sub>2</sub> HgCH(CH <sub>3</sub> ) <sub>2</sub>                                                                                                                                             |
| Tribenzyltin thiosulfate<br>[(C <sub>6</sub> H <sub>5</sub> CH <sub>2</sub> ) <sub>3</sub> Sn] <sub>2</sub> S <sub>2</sub> O <sub>3</sub>                                                       |    | Phenylmercuric myristate<br>C <sub>13</sub> H <sub>27</sub> CO <sub>2</sub> HgC <sub>6</sub> H <sub>5</sub>                                                                                                                                                    |
| Tribenzyltin diallylthallium thiosulfate<br>[(C <sub>6</sub> H <sub>5</sub> CH <sub>2</sub> ) <sub>3</sub> Sn] <sub>2</sub> Tl] <sub>2</sub> S <sub>2</sub> O <sub>3</sub>                      | 25 | p-Amylphenylmercuric laurate<br>C <sub>11</sub> H <sub>23</sub> CO <sub>2</sub> HgC <sub>6</sub> H <sub>5</sub> C <sub>5</sub> H <sub>11</sub>                                                                                                                 |
| Pyridyltellurium thiosulfate<br>(C <sub>5</sub> H <sub>4</sub> NTe) <sub>2</sub> S <sub>2</sub> O <sub>3</sub>                                                                                  |    | Benzylmercuric palmitate<br>C <sub>15</sub> H <sub>31</sub> CO <sub>2</sub> HgCH <sub>2</sub> C <sub>6</sub> H <sub>5</sub>                                                                                                                                    |
| Dicyclohexylgeranium thiosulfate<br>(C <sub>6</sub> H <sub>11</sub> ) <sub>2</sub> GeS <sub>2</sub> O <sub>3</sub>                                                                              | 30 | Tetrahydronaphthylmercuric monatanate<br>C <sub>29</sub> H <sub>59</sub> CO <sub>2</sub> HgC <sub>10</sub> H <sub>11</sub>                                                                                                                                     |
| omega-Chloroamylzinc thiosulfate<br>(ClC <sub>5</sub> H <sub>10</sub> Zn) <sub>2</sub> S <sub>2</sub> O <sub>3</sub>                                                                            |    | Diethylthallium caprylate<br>C <sub>7</sub> H <sub>15</sub> CO <sub>2</sub> Tl(C <sub>2</sub> H <sub>5</sub> ) <sub>2</sub>                                                                                                                                    |
| Nitroxenylarsenic thiosulfate<br>O <sub>2</sub> N.C <sub>6</sub> H <sub>4</sub> C <sub>6</sub> H <sub>4</sub> AsS <sub>2</sub> O <sub>3</sub>                                                   |    | Diphenylthallium succinate<br>[—CH <sub>2</sub> CO <sub>2</sub> Tl(C <sub>6</sub> H <sub>5</sub> ) <sub>2</sub> ] <sub>2</sub>                                                                                                                                 |
| beta-Ethoxyethylselenium thiosulfate<br>(C <sub>2</sub> H <sub>5</sub> OC <sub>2</sub> H <sub>4</sub> Se) <sub>2</sub> S <sub>2</sub> O <sub>3</sub>                                            | 35 | p-Amyloxyphenylthallium didodecanoate<br>C <sub>11</sub> H <sub>23</sub> CO <sub>2</sub> ) <sub>2</sub> TlC <sub>6</sub> H <sub>4</sub> OC <sub>5</sub> H <sub>11</sub>                                                                                        |
| Mercaptophenylaluminum thiosulfate<br>HSC <sub>6</sub> H <sub>4</sub> AlS <sub>2</sub> O <sub>3</sub>                                                                                           |    | Triethyltin adipate<br>[—CH <sub>2</sub> CH <sub>2</sub> CO <sub>2</sub> Sn(C <sub>2</sub> H <sub>5</sub> ) <sub>3</sub> ] <sub>2</sub>                                                                                                                        |
| n-Butylberyllium thiosulfate<br>(C <sub>4</sub> H <sub>9</sub> Be) <sub>2</sub> S <sub>2</sub> O <sub>3</sub>                                                                                   | 40 | Diamyltin divalerate<br>(C <sub>4</sub> H <sub>9</sub> CO <sub>2</sub> ) <sub>2</sub> Sn(C <sub>5</sub> H <sub>11</sub> ) <sub>2</sub>                                                                                                                         |
| II. Organometallic salts of organic acids                                                                                                                                                       |    | p-Aminobenzyltin tributyrate<br>(C <sub>3</sub> H <sub>7</sub> CO <sub>2</sub> ) <sub>3</sub> SnCH <sub>2</sub> C <sub>6</sub> H <sub>4</sub> NH <sub>2</sub>                                                                                                  |
| A. Salts of acyclic acids                                                                                                                                                                       |    | Diphenyllead acid propionate<br>(C <sub>6</sub> H <sub>5</sub> ) <sub>2</sub> Pb(O.CO.C <sub>2</sub> H <sub>5</sub> ) <sub>2</sub> .C <sub>2</sub> H <sub>5</sub> CO <sub>2</sub> H                                                                            |
| Diethylthallium acetate<br>(C <sub>2</sub> H <sub>5</sub> ) <sub>2</sub> Tl.O.CO.CH <sub>3</sub>                                                                                                |    | Diphenyllead trichloroacetate<br>(C <sub>6</sub> H <sub>5</sub> ) <sub>2</sub> Pb(OCOCCl <sub>3</sub> ) <sub>2</sub>                                                                                                                                           |
| Diethylthallium trichloroacetate<br>(C <sub>2</sub> H <sub>5</sub> ) <sub>2</sub> Tl.O.CO.CCl <sub>3</sub>                                                                                      | 45 | Tribenzyltin methyl xanthate<br>CH <sub>3</sub> O.CS.S.Sn(CH <sub>2</sub> C <sub>6</sub> H <sub>5</sub> ) <sub>3</sub>                                                                                                                                         |
| Diphenylthallium acetate<br>(C <sub>6</sub> H <sub>5</sub> ) <sub>2</sub> Tl.O.CO.CH <sub>3</sub>                                                                                               |    | n-Propylmercuric ethyl xanthate<br>C <sub>2</sub> H <sub>5</sub> O.CS.S.HgC <sub>3</sub> H <sub>7</sub>                                                                                                                                                        |
| Tribenzyltin acetate<br>(C <sub>6</sub> H <sub>5</sub> CH <sub>2</sub> ) <sub>3</sub> Sn.O.CO.CH <sub>3</sub>                                                                                   | 50 | Diethylthallium amyl xanthate<br>C <sub>5</sub> H <sub>11</sub> O.CS.S.Tl(C <sub>2</sub> H <sub>5</sub> ) <sub>2</sub>                                                                                                                                         |
| Tribenzyltin dicetylacetate<br>(C <sub>6</sub> H <sub>5</sub> CH <sub>2</sub> ) <sub>3</sub> SnO.CO.CH(C <sub>16</sub> H <sub>33</sub> ) <sub>2</sub>                                           |    | B. Salts of carbocyclic acids                                                                                                                                                                                                                                  |
| Tribenzyltin ethyl succinate<br>(C <sub>6</sub> H <sub>5</sub> CH <sub>2</sub> ) <sub>3</sub> SnO.CO.CH <sub>2</sub> CH <sub>2</sub> CO <sub>2</sub> C <sub>2</sub> H <sub>5</sub>              | 55 | Tribenzyltin cyclohexylcarboxylate<br>C <sub>6</sub> H <sub>11</sub> CO <sub>2</sub> Sn(CH <sub>2</sub> C <sub>6</sub> H <sub>5</sub> ) <sub>3</sub>                                                                                                           |
| Tribenzyltin acetoacetate<br>(C <sub>6</sub> H <sub>5</sub> CH <sub>2</sub> ) <sub>3</sub> SnO.CO.CH <sub>2</sub> CO <sub>2</sub> CH <sub>3</sub>                                               |    | Tribenzyltin phenylacetate<br>C <sub>6</sub> H <sub>5</sub> CH <sub>2</sub> CO <sub>2</sub> Sn(CH <sub>2</sub> C <sub>6</sub> H <sub>5</sub> ) <sub>3</sub>                                                                                                    |
| Tribenzyltin oleate<br>(C <sub>6</sub> H <sub>5</sub> CH <sub>2</sub> ) <sub>3</sub> SnO.CO.C <sub>17</sub> H <sub>33</sub>                                                                     |    | Tribenzyltin octadecylbenzoate<br>C <sub>18</sub> H <sub>37</sub> C <sub>6</sub> H <sub>4</sub> CO <sub>2</sub> Sn(CH <sub>2</sub> C <sub>6</sub> H <sub>5</sub> ) <sub>3</sub>                                                                                |
| Tribenzyltin tartrate<br>[—CHOHCO <sub>2</sub> Sn(CH <sub>2</sub> C <sub>6</sub> H <sub>5</sub> ) <sub>3</sub> ] <sub>2</sub>                                                                   | 60 | Tripropyllead p-ethoxybenzoate<br>C <sub>2</sub> H <sub>5</sub> OC <sub>6</sub> H <sub>4</sub> CO <sub>2</sub> Pb(C <sub>3</sub> H <sub>7</sub> ) <sub>3</sub>                                                                                                 |
| Tribenzyltin dichlorostearate<br>C <sub>17</sub> H <sub>33</sub> Cl <sub>2</sub> CO <sub>2</sub> Sn(CH <sub>2</sub> C <sub>6</sub> H <sub>5</sub> ) <sub>3</sub>                                |    | Triethylgermanium p-nitrobenzoate<br>O <sub>2</sub> N.C <sub>6</sub> H <sub>4</sub> CO <sub>2</sub> Ge(C <sub>2</sub> H <sub>5</sub> ) <sub>3</sub>                                                                                                            |
| Tribenzyltin alpha-amino-n-valerate<br>C <sub>3</sub> H <sub>7</sub> CHNH <sub>2</sub> CO <sub>2</sub> Sn(CH <sub>2</sub> C <sub>6</sub> H <sub>5</sub> ) <sub>3</sub>                          | 65 | Tribenzyltin p-ethoxybenzoate<br>C <sub>2</sub> H <sub>5</sub> OC <sub>6</sub> H <sub>4</sub> CO <sub>2</sub> Sn(CH <sub>2</sub> C <sub>6</sub> H <sub>5</sub> ) <sub>3</sub>                                                                                  |
| Tribenzyltin mercapto-stearate<br>C <sub>17</sub> H <sub>34</sub> (SH)CO <sub>2</sub> Sn(CH <sub>2</sub> C <sub>6</sub> H <sub>5</sub> ) <sub>3</sub>                                           |    | Triamyltin tributylphenylacetate<br>(C <sub>4</sub> H <sub>9</sub> ) <sub>3</sub> C <sub>6</sub> H <sub>2</sub> CO <sub>2</sub> Sn(C <sub>5</sub> H <sub>11</sub> ) <sub>3</sub>                                                                               |
| Tribenzyltin salt of the half-aldehyde of succinic acid<br>H.CO.CH <sub>2</sub> CH <sub>2</sub> CO <sub>2</sub> Sn(CH <sub>2</sub> C <sub>6</sub> H <sub>5</sub> ) <sub>3</sub>                 | 70 | Diethylthallium phenylstearate<br>C <sub>17</sub> H <sub>34</sub> (C <sub>6</sub> H <sub>5</sub> )CO <sub>2</sub> Tl(C <sub>2</sub> H <sub>5</sub> ) <sub>2</sub>                                                                                              |
| Tribenzyltin hydrogen succinate<br>HO <sub>2</sub> C.CH <sub>2</sub> CH <sub>2</sub> CO <sub>2</sub> Sn(CH <sub>2</sub> C <sub>6</sub> H <sub>5</sub> ) <sub>3</sub>                            |    | Pyridylmercuric o-nitrobenzoate<br>O <sub>2</sub> N.C <sub>6</sub> H <sub>4</sub> CO <sub>2</sub> HgC <sub>5</sub> H <sub>4</sub> N                                                                                                                            |
| Tribenzyltin diethoxystearate<br>C <sub>17</sub> H <sub>33</sub> (OC <sub>2</sub> H <sub>5</sub> ) <sub>2</sub> CO <sub>2</sub> Sn(CH <sub>2</sub> C <sub>6</sub> H <sub>5</sub> ) <sub>3</sub> | 75 |                                                                                                                                                                                                                                                                |

|                                                                                                                                                             |    |                                                                                                  |
|-------------------------------------------------------------------------------------------------------------------------------------------------------------|----|--------------------------------------------------------------------------------------------------|
| Tribenzytin cetyl phthalate<br>$C_{16}H_{33}O.CO.C_6H_4CO_2Sn(CH_2C_6H_5)_3$                                                                                |    | Mercurous laurylstannonate<br>$C_{12}H_{25}SnO_2Hg$                                              |
| n-Butylberyllium hydrocinnamate<br>$C_6H_5CH_2CH_2CO_2BeC_4H_9$                                                                                             |    | Mercuric laurylstannonate<br>$(C_{12}H_{25}SnO_2)_2Hg$                                           |
| Tribenzytin cetyl 3-isopropyl-6-methyl- 5<br>3,6 - endoethylene - $\Delta^4$ - tetrahydro-<br>phthalate<br>$C_{16}H_{33}O.CO.C_2H_{18}CO_2Sn(CH_2C_6H_5)_3$ |    | Calcium p-tolylstannonate<br>$(CH_3C_6H_4SnO_2)_2Ca$                                             |
| Tribenzytin 3-isopropyl-6-methyl-3, 6-<br>endoethylene- $\Delta^4$ -tetrahydrophthalate 10<br>$C_{12}H_{18}[CO_2Sn(CH_2C_6H_5)_3]_2$                        |    | Aluminum p-tolylstannonate<br>$(CH_3C_6H_4SnO_2)_2Al$                                            |
| Tribenzytin hydrogen 3 - isopropyl-6-<br>methyl - 3, 6-endoethylene- $\Delta^4$ -tetra-<br>hydrophthalate<br>$C_{12}H_{18}(CO_2H)CO_2Sn(CH_2C_6H_5)_3$      | 15 | Sodium p-tolylstannonate<br>$CH_3C_6H_4SnO_2Na$                                                  |
| beta-Chloroethylarsenic phenylstearate<br>$[C_{17}H_{34}(C_6H_5)CO_2]_2AsC_2H_4Cl$                                                                          |    | Calcium cetylphenylarsenite<br>$C_{16}H_{33}C_6H_4AsO_2Ca$                                       |
| beta-Chloroethyltellurium phenylstea-<br>rate $C_{17}H_{34}(C_6H_5)CO_2TeC_2H_4Cl$                                                                          |    | Calcium p-tert.-amylphenylarsenite<br>$C_5H_{11}C_6H_4AsO_2Ca$                                   |
| Trichloronaphthylmercuric terephthal- 20<br>ate $C_6H_4(CO_2HgC_{10}H_4Cl_3)_2$                                                                             |    | Aluminum p-tert.-amylphenylarsenite<br>$(C_5H_{11}C_6H_4AsO_2)_2Al$                              |
| 2-ethylhexylthallium p-nitrobenzeneazo-<br>p-toluenesulfonate<br>$[O_2N.C_6H_4N=N.C_6H_3(CH_3)SO_3]_2$                                                      |    | Sodium p-tert.-amylphenylarsenite<br>$C_5H_{11}C_6H_4AsO_2Na_2$                                  |
| TICHCH(CH <sub>3</sub> )C <sub>4</sub> H <sub>9</sub>                                                                                                       | 25 | Calcium dipropylarcenate<br>$[(C_3H_7)_2AsO_2]_2Ca$                                              |
| Diethyl $\Delta^4$ -amlytin triamylhydrocinnamate<br>$[C_8H_{11}]_3C_6H_2CH_2CH_2CO_2$                                                                      |    | Aluminum dipropylarsenate<br>$[(C_3H_7)_2AsO_2]_2Al$                                             |
| Tribenzytin cinnamate<br>$C_6H_5CH=CHCO_2Sn(CH_2C_6H_5)_3$                                                                                                  | 30 | Sodium dipropylarsenate $(C_3H_7)_2AsO_2Na$                                                      |
| Furfurylmercuric phenylstearate<br>$C_{17}H_{34}(C_6H_5)CO_2Hg.C_4H_9O$                                                                                     |    | Ammonium laurylstannonate<br>$C_{12}H_{25}SnO_2NH_4$                                             |
| C. Salts of heterocyclic acids                                                                                                                              |    | Ammonium p-tert.-amylphenylarsenite<br>$C_5H_{11}C_6H_4AsO_2(NH_4)_2$                            |
| Tribenzytin furoate<br>$C_4H_3O.CO_2Sn(CH_2C_6H_5)_3$                                                                                                       | 35 | Ammonium dipropylarsenate<br>$(C_3H_7)_2AsO_2NH_4$                                               |
| Furfurylmercuric terpenylate<br>$C_7H_{11}O_2.CO_2HgC_9H_9O$                                                                                                |    | B. Organic salts of organo-metallic acids                                                        |
| Dilaurythallium furfuracrylate<br>$C_4H_3O.CH=CHCO_2Tl(C_{12}H_{25})_2$                                                                                     | 40 | Tetramethylammonium laurylstannonate<br>$C_{12}H_{25}SnO_2N(CH_3)_4$                             |
| omega-Chloroamyl arsenic thiophene-<br>alpha-carboxylate<br>$ClC_5H_{10}As(O.CO.C_4H_3S)_2$                                                                 |    | Tetramethylammonium p-tolystannone<br>$CH_3C_6H_4SnO_2N(CH_3)_4$                                 |
| p-Amyloxyphenylselenium beta-indole-<br>acetate $C_8H_6N.CO_2SeC_6H_4OC_5H_{11}$                                                                            | 45 | Tetramethylammonium cetylphenylar-<br>senite $C_{16}H_{33}C_6H_4AsO_2[N(CH_3)_4]_2$              |
| Tribenzytin tetrahydrofuroate<br>$C_4H_7O.CO_2Sn(CH_2C_6H_5)_3$                                                                                             |    | Tetramethylammonium p-tert.-amyl-<br>phenyl arsenite<br>$C_5H_{11}C_6H_4AsO_2[N(CH_3)_4]_2$      |
| Tribenzytin nicotinate<br>$C_5H_4N.CO_2Sn(CH_2C_6H_5)_3$                                                                                                    |    | Tetramethylammonium dipropylarsenate<br>$(C_3H_7)_2AsO_2N(CH_3)_4$                               |
| n-Butylberyllium nicotinate<br>$C_5H_4N.CO_2BeC_4H_9$                                                                                                       | 50 | Triamylammonium laurylstannonate<br>$C_{12}H_{25}SnO_2NH(C_6H_{11})_3$                           |
| III. Salts of organo-metallic acids                                                                                                                         |    | Triamylammonium p-tolylstannonate<br>$CH_3C_6H_4SnO_2NH(C_6H_{11})_3$                            |
| A. Inorganic salts of organo-metallic acids                                                                                                                 |    | Triamylammonium p-tert.-amylphenyl-<br>arsenite $C_5H_{11}C_6H_4AsO_2[NH(C_6H_{11})_3]_2$        |
| Calcium laurylstannonate<br>$(C_{12}H_{25}SnO_2)_2Ca$                                                                                                       | 55 | Triamylammonium dipropylarsenate<br>$(C_3H_7)_2AsO_2NH(C_6H_{11})_3$                             |
| Sodium laurylstannonate $C_{12}H_{25}SnO_2 Na$                                                                                                              |    | Diethylammonium laurylstannonate<br>$C_{12}H_{25}SnO_2NH_2(C_2H_5)_2$                            |
| Aluminum laurylstannonate<br>$(C_{12}H_{25}SnO_2)_2Al$                                                                                                      |    | Diethylammonium p-tolylstannonate<br>$CH_3C_6H_4SnO_2NH_2(C_2H_5)_2$                             |
| Lead laurylstannonate $(C_{12}H_{25}SnO_2)_2Pb$                                                                                                             | 60 | Diethylammonium p-tert.-amylphenyl-<br>arsenite $C_5H_{11}C_6H_4AsO_2[NH_2(C_2H_5)_2]_2$         |
| Manganese laurylstannonate<br>$(C_{12}H_{25}SnO_2)_2Mn$                                                                                                     |    | Diethylammonium dipropylarsenate<br>$(C_3H_7)_2AsO_2NH_2(C_2H_5)_2$                              |
| Cobalt laurylstannonate<br>$(C_{12}H_{25}SnO_2)_2Co$                                                                                                        |    | Phenylammonium laurylstannonate<br>$C_{12}H_{25}SnO_2NH_3C_6H_5$                                 |
| Nickel laurylstannonate<br>$(C_{12}H_{25}SnO_2)_2Ni$                                                                                                        | 65 | Phenylammonium p-tolylstannonate<br>$CH_3C_6H_4SnO_2NH_3C_6H_5$                                  |
| Ferrous laurylstannonate<br>$(C_{12}H_{25}SnO_2)_2Fe$                                                                                                       |    | Phenylammonium p-tert.-amylphenyl-<br>arsenite $C_5H_{11}C_6H_4AsO_2(NH_3C_6H_5)_2$              |
| Ferric laurylstannonate<br>$(C_{12}H_{25}SnO_2)_3Fe$                                                                                                        | 70 | Phenylammonium dipropylarsenate<br>$(C_3H_7)_2AsO_2NH_3C_6H_5$                                   |
| Stannous laurylstannonate<br>$(C_{12}H_{25}SnO_2)_2Sn$                                                                                                      |    | Phenylammonium ethyl-p-tert.-amyl-<br>phenylarsenite<br>$C_5H_{11}C_6H_4AsO_2(C_2H_5)NH_3C_6H_5$ |
| Stannic laurylstannonate<br>$(C_{12}H_{25}SnO_2)_4Sn$                                                                                                       | 75 | C. Organo-metallic salts of organo-metallic acids                                                |
|                                                                                                                                                             |    | Tribenzytin laurylstannonate<br>$C_{12}H_{25}SnO_2Sn(CH_2C_6H_5)_3$                              |
|                                                                                                                                                             |    | Tribenzytin p-tolylstannonate<br>$CH_3C_6H_4SnO_2Sn(CH_2C_6H_5)_3$                               |

Tribenyltin p-tert.-amylphenylarsenite  
 $C_5H_{11}C_6H_4AsO_2[Sn(CH_2C_6H_5)_3]_2$   
 Tribenyltin dipropylarsenate  
 $(C_3H_7)_2AsO_2Sn(CH_2C_6H_5)_3$   
 Di-omega-chloroamylthallium p-tolyl-  
 stannonate  $CH_3C_6H_4SnO_2Tl(C_6H_{10}Cl)_2$   
 p-tert.-Amylphenylzinc p-tert.-amyl-  
 phenylarsenite  
 $C_5H_{11}C_6H_4AsO_2(ZnC_6H_4C_5H_{11})_2$   
 p-Aminophenylbismuth dipropylarsenate  
 $[C_3H_7)_2AsO_2]_2BiC_6H_4NH_2$   
 Allylselenium laurylstannonate  
 $C_{12}H_{25}SnO_2SeC_6H_5$   
 Mercaptophenylaluminum p-tert.-amyl-  
 phenylarsenite  
 $C_5H_{11}C_6H_4AsO_2AlC_6H_4SH$   
 n-Butylberyllium laurylstannonate  
 $C_{12}H_{25}SnO_2BeC_6H_9$   
 Tribenyltin ethyl-p-tert.-amylphenyl-  
 arsenite  
 $C_5H_{11}C_6H_4AsO_2(C_2H_5)Sn(CH_2C_6H_5)_3$   
 D. Salts of organo-metallic substituted acids  
 Diamylthallium diacetoxymercuri-5-  
 nitrosalicylate  
 $(CH_3CO_2Hg)_2C_6H(OH)(NO_2)CO_2Tl$   
 $(C_5H_{11})_2$   
 Di-(tribenyltin) mercuri-bis-anthrani-  
 late  
 $Hg[C_6H_3(NH_2)CO_2Sn(CH_2C_6H_5)_3]_2$   
 Tribenyltin o-chloromercuribenzoate  
 $ClHgC_6H_4CO_2Sn(CH_2C_6H_5)_3$   
 Tribenyltin o-sulfidomercuribenzoate  
 $S[Hg.C_6H_4CO_2Sn(CH_2C_6H_5)_3]_2$   
 Tribenyltin beta-mercury-bis-pro-  
 pionate  
 $Hg[CH_2CH_2CO_2Sn(CH_2C_6H_5)_3]_2$   
 Tribenyltin alpha-tribenyltinstearate  
 $C_{17}H_{34}[Sn(CH_2C_6H_5)_3]CO_2Sn$   
 $(CH_2C_6H_5)_3$   
 Tribenyltin alpha-diethylthallium-  
 laurate  
 $C_{11}H_{22}[Tl(C_2H_5)_2]CO_2Sn(CH_2C_6H_5)_3$   
 Tribenyltin p-n-butylberylliumben-  
 zoate  
 $C_4H_9BeC_6H_4CO_2Sn(CH_2C_6H_5)_3$   
 Tribenyltin omega-chloroamylarsenic-  
 dibenzoate  
 $ClC_5H_{10}As[C_6H_4CO_2Sn(CH_2C_6H_5)_3]_2$   
 Tribenyltin allylseleniumbenzoate  
 $C_3H_5SeC_6H_4CO_2Sn(CH_2C_6H_5)_3$   
 Aluminum diacetoxymercuri-5-nitro-  
 salicylate  
 $[(CH_3CO_2Hg)_2C_6H(OH)(NO_2)CO_2]_3Al$   
 Calcium beta-mercury-bis-propionate  
 $Hg(CH_2CH_2CO_2)_2Ca$   
 Sodium alpha-tribenyltinstearate  
 $C_{17}H_{34}[Sn(CH_2C_6H_5)_3]CO_2Na$   
 Ammonium alpha-tribenyltinstearate  
 $C_{17}H_{34}[Sn(CH_2C_6H_5)_3]CO_2NH_4$   
 Tetramethylammonium alpha-triben-  
 yltinstearate  
 $C_{17}H_{34}[Sn(CH_2C_6H_5)_3]CO_2N(CH_3)_4$   
 Triamylammonium alpha-tribenyltin-  
 stearate  
 $C_{17}H_{34}[Sn(CH_2C_6H_5)_3]CO_2NH(C_5H_{11})_3$   
 Diethylammonium alpha-tribenyltin-  
 stearate  
 $C_{17}H_{34}[Sn(CH_2C_6H_5)_3]CO_2NH_2(C_2H_5)_2$   
 Phenylammonium alpha-tribenyltin-  
 stearate  
 $C_{17}H_{34}[Sn(CH_2C_6H_5)_3]CO_2NH_3C_6H_5$   
 Tribenyltin tribenyltinsuccinate  
 $(C_6H_5CH_2)_3SnCH_2CH_2CO_2Sn(CH_2C_6H_5)_3$   
 $\downarrow$   
 $CO_2Sn(CH_2C_6H_5)_3$

Any of these compounds or other members of the classes represented may be used within the scope of my invention.

The organo-metallic salts have varying degrees of solubility in hydrocarbon and other oils. In some cases it is necessary to use a solvent for the compound or to form colloidal suspensions of the compound in oil. While some of these compounds have only limited solubility in hydrocarbon oils, it is to be remembered that because of their great efficiency extremely small amounts are often effective. Thus I may use as little as 0.001 per cent of some of these compounds, and it will be seen that a fairly insoluble material may dissolve to a sufficient extent to be satisfactory for my purpose. In general, more than 0.001 per cent of my addition agents are used, and I may add one, two, or even five per cent or more.

Furthermore, it is well known that different types of oils have different capabilities of dissolving a given material. For some purposes therefore, I prefer paraffinic, for other purposes, asphaltic, and for still other purposes, naphthenic or mixed base lubricants. Another method of obtaining a satisfactory mixture of addition agent with the hydrocarbon oil is the use of a mutual solvent to bring the addend into solution. Alternatively, peptizing agents may be added to maintain the organo-metallic salt in permanent suspension.

Many of the more difficult soluble materials are rendered more soluble by the introduction of alkyl groups, particularly those containing four or more carbon atoms. The isoamyl, octyl, lauryl, and octadecyl radicals and radicals from paraffin wax greatly increase the solubility of organic compounds in oil. One or more of such groups may be introduced as required. For example, triphenyltin phosphate is not very soluble in hydrocarbon lubricating oils but tri (cetyl-phenyltin) phosphate is much more soluble.

It will be obvious from these considerations that all the organo-metallic salts are not equivalent and that some are more suitable than others in special cases. Of the examples listed above, for example, the organo-metallic sulfides are likely to be difficultly soluble in petroleum hydrocarbons and fatty oils. Hence, of these, I prefer the purely aliphatic sulfides such as triauryltin sulfide or triamyltin sulfide. If it is particularly desired, however, to use an aromatic organo-metallic sulfide it may best be accomplished by using a compound in which there are at least as many aliphatic carbon atoms as there are aromatic carbon atoms, or more. Thus I prefer to use triquinolyltin triauryltin sulfide or 2-ethyl-hexylphenylzinc sulfide.

In the case of the organo-metallic salts of organic acids, I prefer to use salts of acids having boiling points over 120° C. The salts of the unsubstituted aliphatic acids such as acetic, are less likely to be sufficiently soluble than the trichloroacetates, butyrates, stearates and the like. An exception here, however, are the salts of carbonic acid which may be considered an inorganic acid.

It is sometimes advantageous to combine more than one of these compounds in a blend to obtain particular properties. I accomplish this by mixing two or more of these compounds together and blending the mixture with the hydrocarbon oil or by blending one in the hydrocarbon oil, blending the second into this mixture, and so on until the composition is complete.

The various organo-metallic salts usually improve both the film strength and oxidation characteristics of the hydrocarbon oil. For example, the sludging tendencies may be decreased by as little as 0.001 per cent of my organo-metallic salts compounds. The oxidation characteristics of lubricants are very important, and these are markedly improved by our compounds. The ability to reduce friction is another feature contributed to lubricants by some of our tin compounds.

It may be desirable to include in one and the same blend, in addition to the addends here described, other addends for specific purposes. Thus, I may add a pour point depressor such as a naphthalenechlor wax condensation product, a viscosity index improver such as certain resins or polymerized hydrocarbons, and sulfur or phosphorus containing inhibitors, in addition to my organo-metallic salts. Furthermore, various other metallic compounds may be added to the blend without interfering with the action of my ingredients. Indeed, in some cases it is advantageous to combine with my organo-metallic salts in a hydrocarbon oil blend such materials as calcium dichlorostearate, chromium oleate, aluminum stearate, and other metallic soaps. Various halogenated oxygen bearing ring or aliphatic compounds may be added.

My addends are admirably adapted for use in lubricating oils of all types including those designed for use in automotive crankcases, Diesel oils, and any other oils of lubricating viscosity. Furthermore, my addends are advantageously blended in gasoline and other petroleum fuels either directly or after being blended first in a lubricating oil and then added to the fuel. Soap-thickened mineral oils of all types ranging from those showing only a slight increase in viscosity over that of the mineral oil alone to the semi-solid and solid greases containing fifty per cent or more of soap are amenable to treatment according to my invention. In making these greases, the usual soaps such as sodium stearate, aluminum stearate, calcium soaps of beta fat, and the like may be used to form the large part of the necessary soap. Various other thickening ingredients or materials for other purposes may be added. These include yarn, hair, graphite, glycerol, water, lamp black, mica, zinc, dust, litharge and the like.

Some of these organo-metallic salts are more suitable than others for some purposes. Thus iron and lead compounds, in general, are found to be accelerators of oxidation in crankcase lubricants. On the other hand, these same lead compounds, for example, are quite desirable in the manufacture of mild and violent types of hypoid lubricants. Here the value of the extreme pressure characteristics far overshadows the oxidation accelerating ability.

The following examples of blends of my addition agents are given as illustrations and not as limitations:

#### Example 1

Per cent  
Mid-Continent paraffin base SAE 30 99.0  
Tribenzyltin phosphite 1.0

#### Example 2

Per cent  
California naphthenic base SAE 30 98.7  
omega Chloroamyl diethyltin monothiophosphate 1.3 75 Tribenzyltin phosphite

#### Example 3

|                                                  | Per cent |
|--------------------------------------------------|----------|
| 5 Pennsylvania paraffin base SAE 10              | 99.40    |
| Diethylthallium trichloroacetate                 | 0.05     |
| Naphthalene-chlorwax condensation product        | 0.50     |
| 10 Triamylammonium alpha - tribenzyltin-stearate | 0.05     |

#### Example 4

|                                                  | Per cent |
|--------------------------------------------------|----------|
| 15 Paraffin base bright stock                    | 58.0     |
| Paraffin base neutral oil                        | 40.0     |
| Sulfurized methyl esters of corn oil fatty acids | 0.1      |
| Tribenzyltin stearoylsalicylate                  | 0.2      |
| Calcium dichlorostearate                         | 1.3      |
| 20 Diphenyl-chlorwax condensation product        | 0.4      |

#### Example 5

|                                       | Per cent |
|---------------------------------------|----------|
| 25 Mid-Continent paraffin base SAE 20 | 98.0     |
| Tribenzyltin p-tolylstannonate        | 2.0      |

#### Example 6

|                                                                              | Percent |
|------------------------------------------------------------------------------|---------|
| 30 Mid-Continent mixed base SAE 50                                           | 98.4    |
| Aluminum naphthenate                                                         | 1.3     |
| Tribenzyltin 3-isopropyl-6 methyl-3, 6-en-doethylene-Δ4-tetrahydronphthalate | 0.3     |

#### Example 7

|                                       | Percent |
|---------------------------------------|---------|
| 35 Mid-Continent paraffin base SAE 40 | 93.8    |
| Volatilized corn oil                  | 5.0     |
| Chlorodiphenylene oxide               | 1.0     |
| Trilauryltin phenylstearate           | 0.2     |

#### Example 8

|                               | Percent |
|-------------------------------|---------|
| 40 Naphthenic base SAE 30     | 98.0    |
| Diphenyllead dichlorostearate | 1.3     |
| Methyl dichlorostearate       | 0.7     |

#### Example 9

|                               | Percent |
|-------------------------------|---------|
| 45 Castor oil                 | 98.3    |
| Sulfurized soy bean oil       | 0.2     |
| 50 Dicyclohexylarsenic oleate | 1.0     |
| Chlorodiphenyl                | 0.5     |

#### Example 10

55 In making a grease containing my addends I may use:

|                                     | Percent |
|-------------------------------------|---------|
| 58 Oleic acid                       | 8.1     |
| Lime                                | 1.2     |
| 60 Water                            | 0.3     |
| Dichlorostearic acid                | 1.1     |
| Bright stock                        | 13.1    |
| Distillate (440 seconds at 100° F.) | 76.0    |
| Diamyltin divalerate                | 0.2     |

#### Example 11

In making a lubricating gasoline, I blend 0.5 per cent of the product of Example 1 with gasoline. The product has the composition:

|                           | Percent |
|---------------------------|---------|
| 65 Gasoline               | 99.5    |
| Oil                       | 0.495   |
| 75 Tribenzyltin phosphite | 0.005   |

It will be understood that certain features and sub-combinations may be employed without reference to other species or combinations. This is contemplated by and is within the scope of my claim. It is further obvious that various changes may be made in details within the scope of my claim without departing from the spirit of my invention. It is therefore to be under-

stood that my invention is not to be limited to the details described.

Having thus described my invention, I claim:

5 A lubricant comprising in combination a major proportion of an oil of lubricating viscosity and a minor proportion of diethylarsenic phenyl-stearate.

BERT H. LINCOLN.